

# UNITED STATES PATENT OFFICE

1.943.348

## STEEL FOR NITRIDING

Joseph Kent Smith, Detroit, Mich., assignor to  
The Beryllium Corporation, New York, N. Y.,  
a corporation of Delaware

No Drawing. Application August 10, 1931  
Serial No. 556,326

2 Claims. (Cl. 75—1)

This invention relates to improved metallic compositions of ferrous base subject to nitriding.

It has long been known that certain alloy steels, particularly those relatively low in carbon, when subjected to the action of ammonia gas at elevated temperatures, take on a surface hardness of high magnitude. Such alloy steels have generally contained chromium and aluminum.

10 A series of steels which I have found to be particularly well adapted for nitriding purposes is the group characterized by the simultaneous presence of molybdenum and beryllium, each under 5% of the total. Such steels contain, of course, the usual steel constituents and contaminants—carbon, manganese, sulphur, etc.—and, in addition, the presence of chromium is desirable. An example of a composition which I have found quite suitable for nitriding purposes is a steel containing the following:

|            | Percent |
|------------|---------|
| Manganese  | 0.5     |
| Molybdenum | 0.5     |
| Beryllium  | 0.35    |

Carbon should not exceed 0.5% in the members of this series of my invention, and chromium should not be over 3%.

I claim:—

1 claim. 65

1. A steel for nitriding containing carbon approximately 0.15%, chromium approximately 1.5%, manganese approximately 0.5%, molybdenum approximately 0.5% and beryllium approximately 0.35%, and the balance iron with its common contaminants. 70

2. A steel for nitriding comprising carbon approximately from 0.15% to 0.5%, chromium from 1.5% to 3.0%, manganese about 0.5%, molybdenum from about 0.5% to 5%, beryllium from about 0.35% to about 5% and the balance iron with its common contaminants. 75

## JOSEPH KENT SMITH.

28  80

20 85

Digitized by srujanika@gmail.com

40  95

45 100

50 105

55 110